

Aug. 18, 1925.

1,550,086

C. E. McMANUS

SHEET FOR MAKING CUSHION DISKS AND METHOD OF MAKING SAME

Filed Aug. 29, 1923

Fig. 1.



Fig. 2.



Fig. 3.



Charles E. McManus

INVENTOR

Frank O. Neytrom  
ATTORNEY.

## UNITED STATES PATENT OFFICE.

CHARLES E. McMANUS, OF NEW YORK, N. Y.

## SHEET FOR MAKING CUSHION DISKS AND METHOD OF MAKING SAME.

Application filed August 29, 1923. Serial No. 659,895.

*To all whom it may concern:*

Be it known that I, CHARLES E. McMANUS, a citizen of the United States, residing at the borough of Manhattan, city, county, and State of New York, have invented certain new and useful Improvements in Sheets for Making Cushion Disks and Methods of Making Same, of which the following is a specification, reference being 10 made therein to the accompanying drawings, which form a part thereof.

My invention relates to a sheet of elastic, substantially non-absorbent material composed mainly of cork, which sheet has a 15 thickness which will permit cork disks to be cut therefrom to be used in closure caps for sealing bottles, and to the method of producing same.

It has long been the practice in the manufacture of bottle closures of the crimped metal shell, as well as other types to use cushion disks formed either of natural cork wood, or of composition cork, a material 25 formed of granulated cork waste, the granules of which have been thinly coated with an adhesive or cement before being compacted and bonded to form a homogeneous product.

Because of the extreme care required in 30 selecting the natural cork disks in order to avoid the presence of pores of sufficient magnitude to cause what is known as leakers due to passages at the lip of the bottle, even when a cap containing a disk is applied 35 thereto with considerable pressure; the demand for composition cork disks is progressively increasing so at the present time, it is possibly greater than that for the natural cork. This may be attributed to the 40 fact that composition cork is practically lacking in voids corresponding with the pores of the natural cork, possesses relatively higher elasticity and is of substantially uniform density and elasticity throughout. The 45 composition cork disks have the disadvantage however, of having less durability than the natural cork disk, owing to the tendency of the cork composition to soften when subjected to the action of liquids for a prolonged period and of having a darker color 50 than the natural cork and a tendency to dis- color more rapidly than same.

While such characteristics are present in

composition cork, the life of a disk made therefrom is sufficient to permit its use with 55 many beverages, although, with certain beverages it has been found necessary to apply facing disks of metal, foil, parchment paper or other materials, to the centres of the disk in a position where the material of the disk 60 will be protected from contact with the bottle's contents, the seal however, being made directly against the cork composition, and not against the facing disk.

However, such faced disks require the application of the facing material, centrally of the disks with care and accuracy so as to expose the composition cork about the same in a position where it will seat against the lip of the bottle, and yet not be exposed to 70 contact with the liquid within the bottle.

By my present invention, I am enabled to provide a sheet for making cushion disks, which will have practically all of the advantages of both natural and composition cork 75 disks and practically none of the disadvantages of the latter. Furthermore, this sheet is formed of or includes natural cork of a grade which ordinarily cannot be used in making cushion disks thus permitting the 80 effective utilization of practically all of the cork bark, excepting the outer bark which is so hard and brittle that it possesses none of the properties characteristic of ordinary 85 cork.

In referring to cork of different grades, I have reference not only to the age at which the cork is harvested, but to the different portions of cork, irrespective of its age. The ideal age of cork for use in bottle caps is 90 from six to eight years but generally at this period only one half of the thickness of the cork can be advantageously used, owing to the fact that the fibres at different stages of the development of the cork in process of 95 growth develops pores of progressively increased magnitude toward the outer bark. This outer bark of itself, is so hard, brittle, and irregular as to be practically a waste product. The inner laminations of the cork 100 are substantially free from pores of a depth which will interfere with the use of this portion of the cork in making cushion disks.

The portion of the cork bark adjacent the outer bark has large deep pores therein so 105 that if it be used for cushion disks in bottle

caps, the deformation of the disk when the cap is applied to a bottle will ordinarily be insufficient to close such pores and thus form a perfect seal even when the cork is cut into 5 sheets of one tenth of an inch in thickness. If the cork is cut into thinner sheets most of these sheets will have fairly large openings extending entirely therethrough. For this reason this particular grade of cork is 10 not adapted nor suitable, for use under conditions requiring thin cork substantially free from large surface voids or openings extending entirely therethrough.

By my invention, however, this cork may 15 be effectively used in thin sheets as a surfacing for composition cork sheets since the magnitude of the openings will permit them to be filled or closed by a composition cork backing thus presenting a continuous smooth 20 surface free from voids of a depth which will exceed those in the surface of cork of higher grades. The thinness of the sheets of natural cork will ensure all such voids passing entirely therethrough.

25 It will readily be understood that the number and size of such openings is not great, and that the plasticity of the composition cork, and the pressure used in compacting same, will cause all such openings 30 irrespective of number or size to be effectively filled. Furthermore, the surface of the sheet in all cases, is formed mainly of impermeable natural cork, the small, isolated areas of composition cork being almost 35 indistinguishable from the natural cork. If one of the composition cork fills, should come in contact with the neck of a bottle, it would form a perfect seat thereupon, and being flush with the natural cork surface, 40 would leave no crack or passage at the point. If such a "fill" should occur in a position where it will be exposed to the contents of a bottle the exposed area will not be sufficient to permit any material decomposition 45 of the mass of composition cork backing, or such a distortion thereof as will affect the seal.

50 Discoloration of such areas will not be objectionable because the small areas in each disk are ordinarily few in number and not particularly noticeable.

The invention consists primarily in a sheet for making cushion disks consisting of a surfacing sheet of natural cork 55 having voids extending therethrough, a stratum of composition cork, having portions thereof extending through and filling said voids and having their exposed surfaces substantially flush with the 60 adjacent surface of said natural cork sheet, and an adhesive connecting said surfacing sheet to said stratum; and in such other novel characteristics and in the novel steps and practice in producing said sheet 65 all as hereinafter set forth and described

and now particularly pointed out in the claims hereto appended.

Referring to the drawings:

Fig. 1 is a perspective view of a fragment of a sheet embodying my invention.

Fig. 2 is a cross-sectional view illustrating the method of producing same and

Fig. 3 is a view similar to Fig. 2 showing a different form of the invention.

Like letters refer to like parts through out the several views.

In the embodiment of the invention shown in the drawings, I employ a sheet *a* of natural cork which owing to its having been sliced from the portion of the cork bark adjacent the outer face of the bark will have a number of voids *a'* extending entirely therethrough. The number and size of such voids varies in the same and also in different sheets. The closer the cut is to the outer bark, the greater the number and the larger these voids will be. This variance will also result from differences in age of the cork bark when harvested.

This sheet of cork is backed with a stratum *b* of composition cork or a compacted body formed of granules of cork, thinly coated with a suitable adhesive or cement. This composition as will hereinafter appear, is in a somewhat plastic condition when it is 90 assembled in the sheet and is subjected to heat and pressure during the assembly operation, so that portions *b'* of said backing stratum will extend into and through the voids *a'* so as to completely fill the same. 95 The portions *b'* exposed through said voids will be substantially flush with the adjacent surface of the sheet *a* and form therewith a continuous smooth surface formed mainly 100 of natural cork but having small isolated 105 spots of composition cork varying in size and number throughout the same and different sheets.

Between the natural cork sheets *a* and the backing stratum *b* and the portions *b'* and 110 the edges of the voids *a'* is a suitable adhesive *c* cementing said surfacing sheet and said stratum together. This adhesive may 115 be in the form of a thin stratum applied to the surface of the sheet *a* or to such a stratum applied to the surface of the sheet *a* or to such a stratum expressed from the granular mass forming the stratum *b*.

The embodiment of the invention shown in Fig. 3 differs from that shown in Figs. 120 1 and 2 merely in the respect that the surface of the stratum *b* opposite to that surfaced by the sheet *a* has a facing of paper or other suitable fibrous material cemented to said composition cork stratum by a suitable adhesive *h*. If desired the facing may be provided with gum *g* in a dry state. When this facing *g* is used it will suffice as a paper collet to facilitate bonding of a 125 disk formed from a sheet embodying my 130

invention to its metal shell, this collet, however, forming a substantially integral part of the cushion disk.

Since the face of a disk will be composed in a very large part of a natural cork sheet having a backing of composition cork interposed between it and the metal of the shell, this facing *g* may readily be dispensed with, but is sometimes desirable.

10 In the production of a sheet embodying my invention, I place the sheet *a* of natural cork in a mold *d* and deliver to and distribute substantially equally about said mold, a sufficient quantity of cork granules 15 properly coated with a suitable adhesive to form when compacted, a suitable backing stratum *b* of the desired thickness. If desired, the strip *a* may be coated on that face, with which the cork composition contains, with a suitable adhesive.

Thereafter the mass of composition cork is subjected to a compacting pressure, as by a plunger *e* so as to secure the desired density and thickness of the stratum formed of 25 said mass, and at the same time force, portions *b'* of this mass into and compact them within any voids *a'* occurring in the sheet *a*. While the pressure is thus applied to the contents of the mold, its contents are subjected to heat in any desired manner, as 30 from the burners *f*, for an interval sufficient to set, partially set or properly condition the adhesive contents of the matter within the mold.

35 The sheet is then removed from the mold, the bottom of which will have brought the surface of the sheet *a* and the exposed face of any portion *b'* substantially flush, one with the other.

40 The collet forming facing sheet *g* may be applied during the formation of the composite sheet *a b c* or subsequently as desired.

Cushion disks made from a sheet embodying my invention may properly be considered as but smaller sheets having all of the 45 essential characteristics of the larger sheets. Such sheets are made larger because of economy in production and the absence of difficulties in forming, assembling and handling smaller disks separately.

By producing sheets as described, I am enabled to utilize in very high percentage of cork bark for making satisfactory cushion disks which otherwise could not be used for 55 this purpose. Not only am I enabled to effect this economy, but I can secure a very much increased output of cushion disks from a given quantity of cork bark thus greatly conserving cork bark which is produced in but limited quantities. This saving results in part from the fact that when 60 a facing sheet of natural cork only is used, with a backing of composition cork, the natural cork may be of only one quarter or less thickness than is required for disks

made wholly of natural cork. While the backing stratum *b* is mainly of cork, the granules are produced from cork waste from the manufacture of other articles and does not consume natural cork available for other 70 purposes.

Clean cork waste may be used for making the composition entering into sheets of my invention when a fairly higher grade of cushion disk is to be made. For a lower 75 grade of disk such waste mixed with waste from sheets embodying the invention may be used.

The present invention is designed to utilize for a facing on cushion disks those portions of natural cork which either from the age of the bark when harvested, or from the part of the bark from which the sheet is cut, large voids are inevitable. If such voids are not present in a sheet of cork, such a sheet may be advantageously used by other methods. Hence my present invention permits the utilization of practically all of the cork bark for making cushion disks, excepting 85 the hard brittle outer surface.

Before applying the backing stratum, to the natural cork sheet, it is desirable to remove grit or other small particles therefrom by methods commonly used to clean natural cork when making natural cork disks.

Satisfactory results can be secured by slicing cork bark into sheets of a thickness of forty or more to the inch instead of ten to the inch as when making natural cork disks, so that I am enabled to secure an output of disks having all the desirable surface characteristics of natural cork at least four times that which can be secured when making natural cork disks. This saving is augmented by the condition that the natural cork which I utilize by my present invention will amount to more than 50% of the cork bark in some instances which would otherwise have to be dealt with as waste.

It is not my intention to limit the invention to the details shown in the drawings, since such drawings are merely illustrations of the invention.

The pressure employed may vary, although the thickness of the stratum *b* will permit the desired distribution and compaction of the coated cork granules by a single application of a fairly light pressure and without a tampling action. Any adhesive now commonly used in this art may be employed and the temperature during the application of pressure will be determined by the adhesive used and the time interval required to properly condition such adhesive.

Having described my invention, what I claim as new and desire to have protected by Letters Patent is:—

1. A sheet for making cushion disks consisting of a surfacing sheet of natural cork having voids extending therethrough, a 130

stratum of composition cork having portions thereof extending through and filling said voids and having their exposed surfaces substantially flush with the adjacent 5 surface of said natural cork sheet and adhesive bonding said surfacing sheet to said stratum.

2. A sheet for making cushion disks consisting of a surfacing sheet of natural cork 10 of a thickness to have the elasticity of natural cork and relatively greater flexibility than natural cork of greater thickness, and having voids extending therethrough, a stratum of composition cork 15 having portions thereof extending through and filling said voids and having their exposed surfaces substantially flush with the adjacent surface of said natural cork sheet and adhesive bonding said surfacing sheet 20 to said stratum.

3. A sheet for making cushion disks consisting of a surfacing sheet of natural cork having voids extending therethrough, a stratum of composition cork having portions thereof extending through and filling said voids and having their exposed surfaces substantially flush with the adjacent surface of said natural cork sheet, adhesive bonding said surfacing sheet to said 30 stratum, and a gummed sheet of collet forming material bonded to the opposite side thereof.

4. The herein described method of making a sheet for making cushion disks consisting in applying pressure to a distributed 35

confined mass of cork granules having a coating of adhesive, while in engaging relation to a thin sheet of natural cork having voids therethrough whereby said granules will be compacted and portions thereof will be forced through and compacted in said voids to form a substantially smooth surface outwardly of said sheet and heating the compacted mass and cork sheet while being subjected to pressure, whereby a unitary sheet having a stratum of composition cork and a surface formed of natural cork and isolated spots of composition cork, is formed. 40 45

5. The herein described method of making a sheet for making cushion disks consisting in placing a sheet of natural cork having voids therethrough within a mold, coating the exposed surface of said sheet with an adhesive, delivering and distributing 50 a mass of cork granules coated with adhesive within the mold upon said sheet, applying compacting pressure to said granules whereby portions thereof will be forced and compacted within the voids in 55 said sheet, and applying heat to said mold while the mass therein is held compacted whereby a unitary sheet having a stratum of composition cork and a surface formed of natural cork and isolated spots of composition cork, is formed. 60 65

In witness whereof I have hereunto affixed my signature this 24th day of August, 1923.

CHARLES E. McMANUS.